

## UNITED STATES PATENT OFFICE

2,440,672

## ELECTROPLATING BATH FOR SILVER

Harry J. Green, Indianapolis, Ind., assignor to  
General Motors Corporation, Detroit, Mich., a  
corporation of Delaware

No Drawing. Application October 24, 1942,  
Serial No. 463,250

4 Claims. (Cl. 204—46)

1

This invention has to do with the electrodeposition of metals and has particular application to the electrodeposition of silver.

The primary object of my invention is to provide a new and improved bath and process for the electrodeposition of a metal such as silver in the form of "bright" plate. Other objects and advantages of the invention will become more apparent from the more detailed description which follows.

The invention is based on the use of certain addition agents in novel relationship. The bath or electrolyte of the invention is one of good efficiency and is one that is easy to operate and control. The allowable ranges of current densities, voltages, ranges of the constituents making up the bath and other variables for good deposits are quite broad.

In carrying out the invention an addition agent is provided for the plating bath which may be termed a brightening and structure-controlling agent. When added to plating baths such as the silver-cyanide bath the silver is deposited in the form of bright plate.

The amount of the brightener addition agent is relatively small. Successful results have been obtained with concentrations from 0.05 to 12.5 ml./liter of plating solution. The brightener addition agent is used up or is depleted during operation of the bath and must be replenished.

The brightener addition agents in accordance with the present invention are reaction products of ammonium thiosulfate with various suitable modifying agents. A composition that has proven highly satisfactory is a commercial X-ray fixer used to dissolve silver salts from X-ray film after exposure and development. This solution, hereinafter termed solution A, is composed substantially as follows: ammonium thiosulfate plus ammonium polythionates 32.5%, acetic acid 3.5%, boric acid 3.5%, sodium sulfite 4.2%, water the remainder. The solution has a specific gravity of 1.305 at 25° C. and a pH of 4.25 at 25° C.

Another solution which may be used as the brightener contains in aqueous solution, ammonium thiosulfate (60%) 200 ml., sodium sulfite 7.5 grams, and acetic acid (28%), 28.5 ml. The solution has a specific gravity of 1.311 and a pH of 4.12 at 25° C.

Other acids such as formic, hydrochloric, sulfamic, perchloric, sulfuric are possible for use with the thiosulfate-sulfite mixture but the compounds formed are unstable. However, if bisulfites are added to the thiosulfate, benzoic, tartaric, citric, or hydrocyanic acids will produce effective brightening agents. Acetic and sulfuric acids may also be added to the thiosulfate-bisulfite combination to produce an effective brightener.

Another effective brightener solution is one

2

made by adding 246 ml. of sulfuric acid (7.5%) to 1000 ml. of ammonium thiosulfate (60%).

Other suitable modifying agents which may be added to ammonium thiosulfate to produce effective brighteners are iodine, hypochlorites, or hydrogen peroxide. Iodine, sodium hypochlorite or hydrogen peroxide give very good results when added to ammonium thiosulfate, but the products are not stable. In general the modifying agents for the ammonium thiosulfate may be termed "oxidizing" agents.

The following are illustrative examples of plating baths in which the brightener addition has been used.

## Example I

AgCN, 38-55 g./liter of aqueous solution.  
KCN (free), 38-55 g./liter of aqueous solution.  
Solution A, 0.05-12.5 ml./liter of solution.  
pH, 10.3-14 (12 minimum preferred).

Higher silver cyanide may be used if the free cyanide is increased.

## Example II

AgCN, 100-120 g./liter of aqueous solution.  
KCN (free), 120-150 g./liter of aqueous solution.  
KOH (free), 15-50 g./liter of aqueous solution.  
Solution A, 0.05-12.5 ml./liter of solution.

Silver cyanide concentrations as high as 184 g./liter have been successfully used experimentally.

Equivalent amounts of the other described brightener addition agents may be used in the baths of Examples I and II in place of solution A.

The bath temperature may vary from about 60°-130° F. or higher. At the higher temperatures the current densities may be increased. Using low current densities it is desirable to use low temperatures (about 60°-80°) and low brightener concentrations (0.5-1 ml./liter of plating solution) for maximum brilliancy of deposits. It is highly desirable to control temperatures within 5°-10° F. and preferably somewhat above room temperatures. At present it appears that the best range of temperatures for general work at current densities of 30-75 amps./s. f. cathode area is about 90-130° F.

The current density may be increased greatly by using adequate agitation. Other factors extending the current density range are:

- (a) Addition of potassium hydroxide (15-50 g./liter).
- (b) Increase of temperature to 120-135° F.
- (c) Increase of metal and cyanide in the bath.

Current densities as high as 150 a./s. f. have been obtained with Example I containing 50 g./liter free KOH with effective solution agitation.

The following are illustrative examples of types of agitation which may be employed:

- I. Oscillating rod agitation, 18-50 feet per minute.  
Temperature, 80-100° F.  
Current density, 20-40 a./s. f.  
Brightener, 0.1-0.5 ml./liter of solution.
- II. Cylindrical cathode revolving in solution—  
anode stationary.  
a. Plate deposited on inside of cylinder (anode within cylinder).  
Surface velocity unknown.  
Temperature, 80-120° F.  
Current density, 20-35 a./s. f.  
Brightener, 0.25-1.5 ml./liter.  
b. Plate deposited on outside diameter of cylinder (anode outside cylinder).  
Surface velocity, 20-400 feet/min.  
Temperature, 80-130° F.  
Current density, 20-75 a./s. f. (or more).  
Brightener, 0.25-2 ml./liter of solution.
- III. Cylindrical cathode stationary—anode revolving within it. Plate deposited on inside diameter of cathode.  
Rotation speed, 150-400 R. P. M.  
Temperature, 80-130° F.  
Current density, 20-75 a./s. f.  
Brightener, 0.25-2 ml./liter of solution.
- IV. Anode and cylindrical cathode stationary.  
Solution moving between anode and cathode, parallel to length of cylinder.  
Surface velocity, 20-300 feet/minute.  
Current density, 20-100 a./s. f. (or more).  
Brightener, 0.5-2 ml./liter.

Combinations of the above methods of agitation are also used. In every case best results are obtained with the greatest speed of exposure of the cathode surface to fresh solution without excessive turbulence. In cases IIa and III above, an increased speed of rotation does not necessarily imply a greater exposure of cathode to fresh solution.

Bath voltages vary from 1.2 to 2.8 volts, ordinarily, but depending on current density, distance of anode from cathode, amount of brightener, size of anode and cathode, and composition of bath, may range from 0.8-5 volts.

The brightener addition agent is used up or is depleted during operation of the plating bath. As this occurs more brightener has to be added to maintain the standard of brightness. In one 1200 liter tank 5-20 ml. of brightener are added hourly. This represents about 0.1 to 0.4 ml./liter each 24 hours. If it is wanted to make fewer additions it is possible to add from 0.05 ml. to 4 ml. of brightener per liter of solution, the quantity depending on conditions, and make no further additions until the appearance of the deposits indicates that more is needed. In this case maximum effect of the brightener is attained in about six hours, good results being obtained from the

brightened solution for from 8 to 36 hours, depending upon the amount added, current density, the temperature, and other factors. It is best to add no more brightener than is necessary to give the desired results.

By the use of the bath and process of the invention it is possible to produce in a relatively short time thick deposits of silver in bright form. Current densities as high as 600 amperes per square foot have been used with bath temperatures up to 165° F. Silver has been plated as high as .050" an hour with good agitation.

I claim:

1. A silver cyanide plating bath containing free cyanide and about 0.05 to 12.5 ml. per liter of a solution composed substantially as follows: 32.5% ammonium thiosulfate and ammonium polythionate, 3.5% acetic acid, 3.5% boric acid, 4.2% sodium sulfite, and the remainder water.
2. A silver cyanide plating bath containing free cyanide and to which has been added a brightener addition agent made up substantially as follows: ammonium thiosulfate (60%), 200 ml., an alkali metal sulfite 7.5 grams, and acetic acid (28%), 28.5 ml., said brightener addition agent being present in the plating bath in the proportion within the range .05 to 12.5 ml. per liter of plating solution.
3. A silver-cyanide plating bath comprising essentially an aqueous solution of silver cyanide and an alkali metal cyanide to which has been added 0.05 to 12.5 ml. per liter of a brightener comprising essentially an aqueous solution of ammonium thiosulfate, a compound of the class consisting of alkali metal sulfites and alkali metal bisulfites, and an acid, said brightener having a specific gravity of approximately 1.305 to 1.311 and a pH of approximately 4.12 to 4.25 at 25° C.
4. A silver-cyanide plating bath comprising essentially an aqueous solution of silver cyanide and an alkali metal cyanide to which has been added 0.05 to 12.5 ml. per liter of a brightener comprising essentially an aqueous solution of ammonium thiosulfate, an alkali metal sulfite and acetic acid, said brightener having a specific gravity of approximately 1.305 to 1.311 and a pH of approximately 4.12 to 4.25 at 25° C.

HARRY J. GREEN.

#### REFERENCES CITED

- 50 The following references are of record in the file of this patent:
- UNITED STATES PATENTS
- 55 Number Name Date  
2,110,792 Egeberg et al. Mar. 8, 1938

#### OTHER REFERENCES

- Transactions of the Electrochemical Society, volume 59, 1931, pages 320-335; *ibid.*, volume 80, 60 1941, page 473.
- Treatise on Chemistry, volume I, 1920, page 456, Roscoe and Schorlemmer.